

# UNITED STATES PATENT OFFICE.

JUDSON A. DE CEW, OF MONTREAL, QUEBEC, CANADA.

## SIZING COMPOSITION AND PROCESS OF MAKING SAME.

1,174,697.

Specification of Letters Patent.

Patented Mar. 7, 1916.

No Drawing.

Application filed August 13, 1914. Serial No. 856,618.

*To all whom it may concern:*

Be it known that I, JUDSON A. DE CEW, a citizen of the Dominion of Canada, residing at the city of Montreal, in the Province of 5 Quebec and Dominion of Canada, have invented certain new and useful Improvements in Sizing Compositions and Processes of Making Same, of which the following is a full, clear, and exact description.

10 This invention relates to a sizing composition, particularly adapted for use in the manufacture of paper.

The main object of the invention is to provide a sizing composition with which 15 the paper stock can be treated while in the beating or mixing engine, thereby producing a more waterproof paper than is obtained by the ordinary methods of manufacture.

20 A further object is to provide a sizing composition of such a non-separating character that paper may be waxed or semi-waxed as desired at the time of the sizing operation.

25 A still further object is to provide a sizing composition which will be comparatively inexpensive, requiring only a small proportion of the rosin ordinarily employed.

30 I have discovered that very beneficial results can be obtained by adding to the rosin soap ordinarily used for sizing an unsaponifiable material such as mineral wax, or a difficultly saponifiable material such as 35 wool wax or carnauba wax, which will combine with the free rosin in the size and produce a product with a lower melting point than the ordinary rosin.

In the ordinary method of sizing paper 40 with rosin soap containing unsaponified rosin, the sizing effect is largely obtained by the melting or fusing of the rosin while in the web of paper, by the heat of the drying cylinders. In ordinary practice, however, 45 this result is sometimes not attained on account of the fact that the temperature of the driers is insufficient to melt the free rosin in the size. To overcome this difficulty, I have added to the free rosin soap a

50 certain quantity of wax, which will combine with the free rosin and become substantially permanently incorporated into the soap. It is difficult to emulsify the rosin soap of this character, and proper temperature control is necessary, so that the dilute solutions 55 will not have a temperature in excess of the

melting point of the rosin wax composition. The amount of wax incorporated into the rosin soap will of course vary according to the purpose for which it is required, and the 60 character of the paper being made. When it is only desired to produce efficient sizing results, the amount of wax will be approximately in excess of 15% of the weight of the rosin used, but when it is desired to produce a special waxed or semi-waxed paper, the wax may be used in proportions up to 65 50% of the weight of rosin.

My method of carrying out the process is to add to the free rosin soap the quantity 70 of waxed desired, and then to emulsify same by means of a process for producing size solutions, such as that described in U. S. Patent, Reissue No. 12,549. This size solution is mixed with the paper stock 75 while in the beating or mixing engine, and thus a waxed or semi-waxed paper may be produced without putting the stock through the ordinary steps of a waxing process. With this product, I am able to 80 size paper more efficiently than with a rosin soap alone, and by the use of an amount of wax up to the maximum that can be emulsified, various papers can be produced intermediate in character between a waxed paper 85 and a rosin sized paper. This class of paper will be found just as suitable for waterproof bottles, cups, and other waxed paper articles as if made from paper which was originally rosin sized and afterward 90 immersed in molten wax. I am therefore able to produce a waxed or semi-waxed paper which is absolutely waterproof, and which has never before been produced by this process.

95 In fact, the surface of the paper will be improved by this process, as when ordinary rosin soap is used, the sizing is injured during the calendering operation on account of the brittleness of the rosin, whereas this sizing composition is more pliable and adjusts itself to the molding of the calenders. I also find that the presence of wax in the size composition makes it less reactive to the injurious effects of chemical residues and gives a more colloidal precipitate with alum or other precipitating agent.

100 Having thus described my invention, what I claim is:—

110 1. A non-separating composition consisting of permanently emulsified rosin and wax in which the wax is in excess of 15% of the weight of the rosin.

2. A non-separating sizing composition consisting of permanently emulsified rosin and a mineral wax in which the wax is in excess of 15% of the weight of the rosin.
- 5 3. A non-separating composition consisting of permanently emulsified rosin and a difficultly saponifiable wax in which the wax is in excess of 15% of the weight of the rosin.
- 10 4. A process of making non-separating water-proof sizing composition which con-

sists in permanently emulsifying wax and rosin when the wax is in excess of 15% of the weight of the rosin, for the treatment of paper stock in the beating engine.

In witness whereof, I have hereunto set my hand, in the presence of two witnesses,

JUDSON A. DE CEW.

Witnesses:

S. R. W. ALLEN,  
G. M. MORELAND.